

# UNITED STATES PATENT OFFICE.

JOSEPH BYRON BESSEY, OF LONDON, ENGLAND.

## PROCESS FOR PRODUCING FUEL FROM PEAT BY MEANS OF THE ELECTRIC CURRENT.

No. 817,899.

Specification of Letters Patent.

Patented April 17, 1906.

Application filed October 5, 1905. Serial No. 281,590.

*To all whom it may concern:*

Be it known that I, JOSEPH BYRON BESSEY, gentleman, residing at London, England, have invented a new Process for Producing 5 Fuel from Peat by Means of the Electric Current, of which the following is a specification.

The invention refers to a process for producing a fuel from peat, the peat being between the poles of an electric circuit, so that the circuit is closed by the mass. The known processes of this kind frequently depend on the electrothermic action of the electric current. They thus either intend to 15 evaporate the water contained in the peat by the heating effect of the electric current or to carbonize even the peat by the same heating effect of the current. For these processes it is of course of no importance if the current 20 employed be continuous or alternating, as only the heating effect is of importance. Naturally, however, these processes will be very expensive, owing to the strength of the current required and the length of time it has 25 to work. Furthermore, even if only the water is to be removed the peat is always heated above 100° centigrade (212° Fahrenheit,) but at this temperature already the valuable component parts of the peat commence 30 to be decomposed. The fuel thus loses of heating value, and above all the organic agglutinants contained in the peat are lost partly, so that a self-hardening of the thus-treated peat cannot or at least only very im- 35 perfectly take place, and a strong compression becomes necessary to produce solid peat-coal or peat briquets. A second style of treating raw peat by means of the electric current consists in the physical phenomenon 40 called "electro-osmosis"—viz., the migration of particles of liquids, owing to the influence of the electric current or in the electrolytical disintegration of water, respectively. For this kind of process of course the use of con- 45 tinuous current is the main condition, as alternating current cannot effect at all electro-osmosis and electrolysis. Besides the fact that continuous current is expensive in use in this kind of process the peat also is partly 50 decomposed in its organic components. Above all, the organic agglutinants contained in the peat are disintegrated, owing to the electrolysis, which will always come to effect when continuous current is applied. Therefore, it is necessary when using these processes to compress the peat after the electric

treatment in order to obtain solid pieces or briquets.

The present invention has the purpose to obtain in a cheap manner a dry peat-coal which will offer without any compression merely by self-hardening a fuel of high value and capable of being transported. According to the invention this purpose is obtained by the combination of, first, employing such current as will avoid electrochemical disintegration of the organic agglutinants—viz., alternating current—and, second, by regulating this current in its action in such a manner that no heating up to 100° centigrade (212° Fahrenheit) in the stuff will take place. In this way any decomposition of the organic agglutinants is avoided. The consequence is that peat treated in such a manner and after the water freed by the electric current has been removed will harden by itself in the air, contracting at the same time, so that no compression is required to obtain solid briquet-like pieces.

The voltage and strength of the alternating current sent through the peat, also the length of time during which the current must act, depends on the amount of solid parts contained in the peat. The process has been found to be very easily and cheaply carried out when an alternating current of two hundred volts and twelve hundred amperes per ton of solid parts contained in the raw peat is employed for two periods of each five minutes, whereat the water freed by the effect of the electric current is mechanically removed after each period of treatment. During its action the current is regulated in such a manner that a heating of the peat above 100° centigrade (212° Fahrenheit) is avoided.

The whole process thus for producing a solid fuel from peat according to the present invention is, for instance, as follows: The raw freshly-cut peat is freed in presses, centrifuges, or similar appliances from the water mechanically contained in it and then placed between the poles of an alternating-current circuit. Now an alternating-current of two hundred volts and twelve hundred amperes per ton of solid material contained in the peat is sent through the peat for five minutes. The hereby-freed water is instantly removed again by presses, centrifuges, or the like. Now again an alternating current of corresponding voltage and strength is sent through the peat for the same length of time, and the hereby-freed water is again mechan-

ally removed. When stored in the air after mixing in a kneading apparatus or the like, the thus-treated peat will harden by itself, shrinking considerably and form a solid coal-like fuel of high heating value, owing to the fact that the organic agglutinants liberated by the influence of the alternative current are distributed in an undisintegrated condition throughout the peat mass.

10 What I claim, and desire to secure by Letters Patent, is—

Process for producing a fuel from peat by means of the electric current, consisting in exposing the peat, previously freed from water by mechanical means, to the effect of an

alternating current of two hundred volts and twelve hundred amperes per ton of solid material contained in the peat, for some periods, the current being regulated in such a manner, that a heating of the peat above 100° <sup>20</sup> centigrade is avoided, and removing the water freed by the action of the alternating current after each charge of electricity.

In testimony whereof I have hereunto set my hand in presence of two subscribing witnesses.

JOSEPH BYRON BESSEY.

Witnesses:

H. D. JAMESON,  
F. L. RAND.